

1

2,978,292

## MANUFACTURE OF RAYON

Pieter Coenraad Limburg, Arnhem, Aart Buurman, Velp, and Robbert Aldert Vroom, Arnhem, Netherlands, assignors to American Enka Corporation, Enka, N.C., a corporation of Delaware

No Drawing. Filed July 9, 1958, Ser. No. 747,360

Claims priority, application Netherlands July 13, 1957

6 Claims. (Cl. 18—54)

This invention relates to the manufacture of viscose rayon and more particularly to an improved process for making rayon and to an improved viscose spinning solution.

In Dutch patent application Serial No. 195,721 a process is described for the manufacture of artificial threads, fibers and like products from viscose, in which a viscose solution containing polymers of an epoxyalkane in quantities of 0.1—1% by weight (calculated on the viscose) is spun in a sulfuric acid spinning bath. The bath contains at least 2% zinc sulfate and, in percentage by weight, the  $H_2SO_4$  content of the bath does not exceed 1.3 times the alkali content of the viscose.

By means of this process threads are obtained which show a so-called skin structure. Consequently the swelling value of these threads is low and the double loop strength as well as the resistance to abrasion are high. These threads are very suitable for the manufacture of tire cord. Staple fibers similarly made may be especially used in those cases where a satisfactory resistance to washing is required.

In the processing to cord a number of threads are combined and twisted together. It is known that during this process twisting losses occur, i.e. the strength of the manufactured cord is less than the sum of the strengths of the composite threads. These twisting losses will hereinafter be called cord losses.

It has already been previously found—as described in Dutch patent application Serial No. 197,805—that by using epoxyalkane polymer having a specific composition and molecular weight, namely by using polymers of epoxyethane having a molecular weight of between 3800 and 4200, the cord loss may be reduced.

It has now been found that by using a combination of the polymers of the epoxyalkane with certain amines in a specific ratio the cord loss may be even further reduced.

It is an object of this invention to provide a method for making rayon yarn having improved physical properties by utilizing a novel combination of modifiers.

Another object is to provide a new viscose spinning solution.

Other objects will be apparent from the following detailed description.

The present invention consists of a process of spinning into an acid spinbath a viscose solution that contains, in addition to the epoxyalkane polymers, also one or more compounds of the general formula:



in which R is an aliphatic chain having at least 8 C-atoms, in which n is 2, 3 or 4 and x+y is at least 2, while neither x nor y may be zero, the quantity of the substituted amines amounting to 15 to 40% by weight of the total amounts of the epoxyalkane polymer and the amine.

2

It is also part of the invention to provide a new viscose spinning solution containing the above mentioned materials.

In general, substituted amines are used in which R consists of an aliphatic chain having 8 to 24 carbon atoms. Amines in which n equals 2 may be considered for use. The total number of  $(C_nH_{2n}O)$ -units in the amines used preferably lies between 5 and 25.

However, amines to which a higher number of

10  $(C_nH_{2n}O)$ -units

have been bound may also be considered for use.

Examples of amines of the formula:



are the products marketed under the names of Ethomeen C/15, Ethomeen C/20, Ethomeen C/25, Ethomeen C/60, Ethomeen S/15, Ethomeen S/20, Ethomeen S/25, Ethomeen S/60, Ethomeen T/15, Ethomeen T/20, Ethomeen T/25, Ethomeen T/60 and Hüls V 1011 T.

The Ethomeens are prepared by reacting amines derived from higher fatty acids with ethylene oxide. In this way the C-Ethomeens are derived from coconut oil, the S-Ethomeens from soybean oil and the T-Ethomeens from tallow. The numbers 15, 20, 25 and 60 following on the capitals indicate, after a deduction by 10, the number of ethylene oxide molecules which have reacted with 1 molecule of the amine.

Hüls V 1011 T is a representative of the group of compounds of the formula:



in which R represents an alkyl radical having 8 to 24 C-atoms, (x+y) has a value of between 5 and 25 and neither x nor y are zero.

40 If the aforementioned amines together with epoxyalkane polymers in the stated amounts of 15 to 40% by weight, calculated on the mixture of the epoxyalkane polymers and the amines, are added to viscose, said amines reduce the cord losses which up till now occurred when using only epoxyalkane polymers. It seems that this should be attributed to the fact that these amines give the threads a smoother surface. When using only the epoxyalkane polymers said surface namely is rather rough.

45 The smoother surface means that also the dirt-adhering capacity is smaller so that after the threads have been cut to staple they are very suitable to be used as rug fibers.

50 The correct amount of the nitrogen-containing compound within said range depends on the structure of the amine, as well as on the epoxyalkane polymer used.

For instance, when using polypepoxyethane having a molecular weight of 3000 it is preferred to use the commercial product Hüls V 1011 T in an amount of 25% by weight (calculated on the total weight of the poly-epoxyethane and the amine). The epoxyalkane polymers which are used in combination with the above-mentioned nitrogen compounds may be straight polymers, copolymers or so-called block polymers of epoxyalkane or substitution products thereof. The epoxy compounds from which the polymers used are prepared have the general formula:



55 70 in which R represents hydrogen, an alkyl group, a cycloalkyl group or an aryl group. Examples thereof are

epoxyethane and epoxypropane. An example of a block polymer is  $\text{HO}(\text{C}_2\text{H}_4\text{O})_a(\text{C}_3\text{H}_6\text{O})_b(\text{C}_2\text{H}_4\text{O})_c\text{H}$ , in which  $b$  equals 30 and  $a+c$  equals 85. Of these polymers an amount of between 0.2-0.5% by weight, calculated on the viscose, is in general added to the spinning solution.

With an amount of 0.2% by weight of polyepoxyalkane the amount of the amine lies approximately between 0.04 and 0.11% by weight. If used in unmixed condition these amounts do not give rise to the formation of threads with a skin character. If larger amounts of the epoxyalkane polymer and higher mixing ratios between the amine and the epoxyalkane polymer are used the concentration of the nitrogen compound enters the range where the latter compound itself causes the production of threads with a skin character, but in that case the effect is achieved that in processing the threads to cord, losses become lower than without the use of said nitrogen compounds.

It is preferred to use amounts of the nitrogen-containing substance which lie in the lower percentages of the indicated range. This has the advantage that when regenerating the spinning bath, which is carried out under evaporation, as well as when deaerating viscose before spinning, an inconvenient formation of foam is avoided to a considerable degree.

Although it is possible to operate with spinning baths having a sulfuric acid content of 10% by weight and higher, it has been found preferable, in connection with the properties of the threads, such as the strength and the swelling in water, to operate with spinning baths in which the sulfuric acid content is less than 7% by weight.

The zinc sulfate content in the spinning baths may vary considerably above the minimum of 2% by weight and may amount for example, to 10% by weight and higher. For economic reasons the lower percentages deserve preference.

The drawing which is necessary to obtain threads having the required properties may be carried out in a so-called one-bath process as well as in a second bath and in one or more stages.

When the drawing operation is carried out in a second bath this is, as usually, arranged so that at the end of the drawing process the cellulose xanthate is decomposed to a considerable degree, preferably to a cellulose xanthate ratio of maximum 0.02.

By the xanthate ratio, which is determined according to the method also known for the determination of the gamma number, is meant the ratio between the number of the xanthate radicals still present and the total number of the glucose radicals ( $\text{C}_6\text{H}_{10}\text{O}_5$ ).

The invention will be further explained with reference to the following examples which are to be regarded by no means as restrictive. In these examples the composition of the viscose, the spinning bath, etc., is expressed in percentages by weight.

#### Example I

A viscose spinning solution was prepared with a cellulose content of 5.5% and an alkali content of 3.8%, calculated on the viscose, as well as 0.15% polyethylene oxide having a molecular weight of about 4000 and also 0.05% of the product marketed under the name of Hüls V 1011 T. This solution was spun at a xanthate ratio of 0.48 and a viscosity of 70 sec. (falling ball test) into an aqueous spinning bath at 46° C. containing 3.2% sulfuric acid, 12.0% sodium sulfate and 6.0% zinc sulfate. In the spinning bath the freshly spun thread was immersed for a distance of 95 cm., passing through a two diameter tube. The first portion of the tube had a length of 55 cm. with a diameter of 20 mm. and the second portion a length of 30 cm. with a diameter of 30 mm. The thread was drawn 45% in the atmosphere and then drawn 50% in a second bath containing 3%  $\text{H}_2\text{SO}_4$  and less than 2% salts. The temperature of the

second bath was 95° C. The length of immersion in the second bath was 150 cm. The speed at which the thread was then collected on a spool amounted to 62 m./min. The thread obtained was thereafter washed free from acid in the usual manner, sized and dried under tension after which the properties were determined. The thread, which had a total denier of 1656 and consisted of 1000 filaments, was then found to have a swelling value of 68%. The double loop strength and the resistance to abrasion were excellent. The cord loss amounted to 16%, whereas without the addition of the nitrogen compound the cord loss amounted to 24%.

#### Example II

15 A viscose having a cellulose content of 7.3% and a sodium hydroxide content of 5.5%, and containing 0.11% of polyethylene oxide having a molecular weight of 3000 as well as 0.04% of the substance marketed under the name of Ethomeen C/25, was at a xanthate ratio of 0.45 and a viscosity of 60 sec. (falling ball test) spun through a spinneret having 1000 orifices of 60 microns into a spinning bath at 49° C. containing 5.2% sulfuric acid, 13.0% sodium sulfate, 4.5% zinc sulfate and 0.05% laurylpyridinium sulfate.

20 25 After leaving the spinning bath in which the freshly spun threads passed through a tube of the shape and dimensions stated in Example I and in which the length of immersion was 110 cm., the freshly spun threads were drawn 100% in a second bath having a length of travel of 120 cm. and containing 2.5% sulfuric acid at 95° C.

30 35 After the drawing process the threads were collected in a spinning pot at a speed of 60 m./min. and were thereafter washed, after-treated and dried in the known manner.

35 The threads thus produced had a swelling value of 67%. On processing to cord the cord loss amounted to 18% whereas under similar conditions but without using Ethomeen C/25 this loss amounted to 26%.

40 What is claimed is:

1. A method of producing viscose rayon comprising the steps of spinning a viscose solution having incorporated therein 0.1-1.0% of an epoxyalkane polymer of the class consisting of epoxyethane polymer and epoxypropane polymer of a molecular weight of about 3000 and 45 a compound of the general formula



50 in which  $\text{R}$  is an aliphatic chain having at least 8 carbon atoms,  $n$  is 2, 3, or 4, and  $x+y$  is at least 2 with neither  $x$  nor  $y$  being zero, into an acid coagulating bath the quantity of the substituted amine being 15-40% by weight of the total amount of the epoxy alkane polymer and the amine compound.

55 60 2. The process of claim 1 wherein the epoxyalkane polymer is epoxyethane polymer.

3. The process of claim 1 wherein the acid coagulating bath is a sulfuric acid bath containing at least 2% by weight of zinc sulfate.

65 4. The process of claim 1 wherein the substituted amine compound added has the formula



70 75 in which  $\text{R}$  is an alkyl radical having 8-30 carbon atoms,  $x+y$  has a value between 5 and 25 with neither  $x$  nor  $y$  being zero.

5. The process of claim 3 wherein the concentration of the sulfuric acid in the coagulating bath is 70% or less.

6. A viscose spinning solution containing 0.1-1.0% by

weight of a polymer of an epoxyalkane of the class consisting of epoxyethane polymer and epoxypropane polymer of a molecular weight of about 3000 to about 4000 and a compound having the general formula



in which R is an aliphatic chain having at least 8 carbon atoms, n is 2, 3, or 4, and x+y is at least 2 with neither x nor y being zero, the quantity of the substituted amine

being 15-40% by weight of the total amount of the polymer of an epoxyalkane and the amine compound.

References Cited in the file of this patent

UNITED STATES PATENTS

|            |                  |                |
|------------|------------------|----------------|
| Re. 24,486 | Mitchell         | June 10, 1958  |
| 2,572,217  | Thurmond         | Oct. 23, 1951  |
| 2,593,466  | MacLaurin et al. | Apr. 22, 1952  |
| 2,696,423  | Dietrich         | Dec. 7, 1954   |
| 2,852,333  | Cox et al.       | Sept. 16, 1958 |
| 2,852,334  | Hollihan et al.  | Sept. 16, 1958 |

UNITED STATES PATENT OFFICE  
CERTIFICATION OF CORRECTION

Patent No. 2,978,292

April 4, 1961

Pieter Coenraad Limburg et al.

It is hereby certified that error appears in the above numbered patent requiring correction and that the said Letters Patent should read as corrected below.

Column 3, line 33, for "minimlm" read -- minimum --;  
line 37, for "therads" read -- threads --; same column 3,  
line 68, for "frshly" read -- freshly --; column 4, line 6,  
for "th eproperties" read -- the properties --; line 74, for  
"70%" read -- 7% --.

Signed and sealed this 15th day of August 1961.

(SEAL)

Attest:

ERNEST W. SWIDER

Attesting Officer

DAVID L. LADD

Commissioner of Patents